

Patented May 5, 1925.

1,537,047

# UNITED STATES PATENT OFFICE.

MAURICE E. LOUTH AND ARTHUR WHITE YOUNG, OF KOKOMO, INDIANA, ASSIGNEES  
TO UDYLITE PROCESS COMPANY, OF KOKOMO, INDIANA, A CORPORATION OF IN-  
DIANA.

## CADMUM PLATING.

No Drawing.

Application filed June 5, 1924. Serial No. 718,155.

To all whom it may concern:

Be it known that we, (1) MAURICE E. LOUTH and (2) ARTHUR WHITE YOUNG, citizens of the United States, residing at 5 Kokomo, in the county of Howard and State of Indiana, have invented certain new and useful Improvements in Cadmium Plating, of which the following is a specification.

We have found in electroplating with cadmium that it is possible to vary and coordinate the various factors involved, to wit, the composition of the bath, the type of anode, the ratio of active to inactive anode surface, the ratio of anode to cathode surface, the use of brightening or addition agents, and the current density in such a way as to produce a number of desirable results, among which may be mentioned the maintenance of the electrolytic bath at maximum efficiency over a long period of time and the production of coatings having the desired characteristics.

The most important factor in the present invention is the bath composition. In referring to bath composition, we do not mean to indicate the kind of chemical substances involved but rather the relation of the chemical substances in the bath to each other. We employ a sodium cadmium cyanide bath which may be prepared, for instance by dissolving cadmium oxide or hydrate or carbonate in an aqueous solution of sodium cyanide. The resulting bath contains (1) sodium cadmium cyanide, (2) sodium hydroxide in case cadmium oxide or hydrate is used in preparing the bath or sodium carbonate in case cadmium carbonate is used in preparing the bath, and (3) sodium cyanide used in excess of that required to convert the cadmium oxide, hydrate or carbonate to sodium cadmium cyanide. The composition of the sodium cadmium cyanide bath may vary rather widely. For example, it may contain from  $\frac{1}{4}$  to 6 ounces of cadmium per gallon and from  $2\frac{1}{2}$  to 6 ounces of free sodium cyanide per gallon. By "free sodium cyanide" is meant the sodium cyanide used in making up the bath in excess of that which is used in converting the cadmium oxide, hydrate or carbonate dissolved therein to sodium cadmium cyanide. The free sodium cyanide content of the bath may, when insoluble anodes are employed in the plating process, go as low as  $\frac{1}{4}$  ounce per gallon,  $2\frac{1}{2}$  ounces per gallon

being the lower limit when cadmium anodes are used, and on the other hand may go above 6 ounces up to say 10 ounces per gallon, but since a free sodium cyanide content above 6 ounces per gallon is without apparent effect it is undesirable from an economical standpoint. The sodium hydroxide or carbonate content of the bath resulting from the interaction of the sodium cyanide with the cadmium oxide, hydrate or carbonate of course, unless extra sodium carbonate or hydroxide is added, will be chemically equivalent to the quantity of cadmium oxide, hydrate or carbonate dissolved, and although we do not regard the addition of extra sodium carbonate or hydroxide to the bath as being advisable, such additions are not to be regarded as a departure from our invention.

A bath suitable for commercial use may be prepared as follows: To a water solution of sodium cyanide containing about  $8\frac{3}{4}$  ounces of sodium cyanide per gallon there is added about  $2\frac{1}{2}$  ounces of cadmium oxide per gallon. The cadmium oxide dissolves completely, giving a solution containing about 5 ounces of free sodium cyanide and about 2 ounces of cadmium per gallon.

As is indicated above, the limits stated for the free sodium cyanide content of the bath are not merely arbitrary limits but have a definite relation to the results to be produced. In the same way the range of cadmium content of the bath specified bears a definite relation to the results to be produced. At below  $\frac{1}{4}$  ounce of cadmium per gallon of electrolyte the bath is difficult to maintain, while at above 6 ounces per gallon there is a tendency, when electroplating at average current density to be described hereinafter, for the electrodeposit to tree. A cadmium content of about 2 ounces per gallon therefore is preferred, since we have found in practice that this content gives good coatings and is easily maintained and the tendency to deviate from this content beyond either limit is the minimum.

The cadmium oxide, hydroxide or carbonate used in making up the bath should be pure and particularly with reference to thallium, tin and lead which we have found to cause undesirable deposits. Lead in quantities as small as 0.1% of the cadmium causes serious trouble.

The anodes to be used with the above de-

scribed sodium cadmium cyanide bath may be wholly inactive, for instance, all steel, or wholly active, that is, pure cadmium, or a combination of active and inactive material, 5 for instance a combination of steel and metallic cadmium in a definite ratio to each other, which ratio bears a definite relation to the bath composition, as will appear hereinafter.

10 With a sodium cadmium cyanide bath as described above and within the limits of current density and anode to cathode ratio to be described hereinafter, there may be used either all cadmium anodes, or all inactive 15 anodes such as steel or anodes made up of both cadmium and steel or other inactive material in varying proportions. At the lower limit of free sodium cyanide content, that is at  $\frac{1}{4}$  ounce per gallon and up to  $2\frac{1}{2}$  20 ounces per gallon, inactive anodes such as steel or carbon may be used. The use of inactive anodes, however, is not preferred, because it requires for the maintenance of the bath suitable additions of cadmium, and 25 besides, particularly when graphite anodes are used, it appears that the cyanide radical is gradually broken up, resulting in a decrease in the cyanide content of the bath which requires occasional additions of 30 sodium cyanide, and further there is a gradual formation of sodium carbonate in the bath which eventually makes necessary its purification or replacement.

If pure cadmium anodes are used, the 35 free sodium cyanide content of the bath must be maintained at or above  $2\frac{1}{2}$  ounces per gallon, otherwise polarization takes place with a corresponding diminution in plating values. At above  $2\frac{1}{2}$  ounces of free 40 sodium cyanide per gallon with pure cadmium anodes the cadmium content of the bath tends to increase. The use of pure cadmium anodes is not preferred, because it is difficult and troublesome to maintain 45 the free sodium cyanide content of the bath at such a figure, about  $2\frac{1}{2}$  ounces per gallon, that neither polarization or too great a building up of the cadmium content of the bath will occur. We therefore prefer the 50 use of combined soluble and insoluble anodes, the active and inactive surface of which may be varied in a bath containing  $2\frac{1}{2}$  ounces or more of free sodium cyanide per gallon. The ratio of active to inactive 55 surface in the combination soluble and insoluble anodes varies widely, depending upon the composition of the bath and other factors within the limits heretofore defined. It is impossible to state a general rule for 60 the determination of the best ratio of active to inactive anode surface under all or any specific set of conditions. The preferred ratio must be determined by experiment in each particular case. The following specific 65 example is illustrative:

In a 500 gallon plating bath in continuous operation containing on an average about 2 ounces of cadmium and about 5 ounces of free sodium cyanide per gallon, in the use of which a cathode surface to anode surface 70 ratio of from  $1\frac{1}{2}$ -1 to 1-1 was maintained, an active to inactive anode surface ratio of 45 to 55 gave satisfactory results. In the use of this bath the cadmium content of the bath was found to vary within  $\frac{1}{4}$  ounce per 75 gallon above and below the average cadmium content and the losses of sodium cyanide were very small, a few pounds per month. In general it may be stated that the active to inactive anode surface ratio may vary 80 from about 1-3 to about 3-1.

The current density which may be used along with the other factors, and particularly with reference to the bath composition defined, may vary from 4 to 100 amperes per 85 square foot. However, when a brightening agent is used as described below, the upper limit of current density is about 30 amperes per square foot, above which limit the coatings become less lustrous and more gray as 90 the current density increases.

The plating may be carried out either in the presence or absence of addition or brightening agents, but the use of addition agents is preferred. If addition agents are 95 not used the coatings may be either dull white, silver white or gray, depending upon the current density. Such coatings are soft and are apt to be cut through by buffing, but they are satisfactory for some classes of 100 rough work such as castings. The use of addition agents is practically indispensable for various classes of work such as that upon which a high polish is desired, or which is to be color-buffed or over-coated with nickel. 105 By the use of addition agents the coatings are made physically harder and denser and given a bright lustrous sheen. Such coatings produced with the use of addition agents in many cases have sufficient luster 110 so that the use of other finishes is unnecessary. They may be buffed without cutting through and are more resistant to blows and scratches and more continuous when tested for pin holes than coatings made without 115 the use of addition agents.

Various addition agents may be used, but we prefer the use of milk or protein addition agents, such as wool and casein. Of wool from  $\frac{1}{2}$  to 10 grams per gallon of 120 electrolytic bath may be used, about  $1\frac{1}{2}$  grams being the usual average. The wool may be added to the plating bath by dissolving it in concentrated warm caustic soda solution and adding this solution to the 125 bath. Casein may be used in quantities varying from  $\frac{1}{2}$  to  $2\frac{1}{2}$  grams per gallon. Casein is added in the form of a solution in warm dilute aqua ammonia. Milk is the preferred addition agent and is used prefer- 130

ably in the form of the so-called evaporated milk which is an unsweetened product made by evaporating whole milk under vacuum to about one-half its original volume. Evapo-  
5 rated milk may be used in quantities vary-  
ing from 5 to 40 cc. per gallon, a satisfac-  
tory average amount being 10 cc. per gallon.  
Our invention therefore involves gener-  
ally the determination and coordination of  
10 the various factors involved in electroplating  
cadmium from cyanide solutions and more  
particularly the determination of the rela-  
tions of the various factors involved such  
as bath composition, active to inactive anode  
15 surface ratio, anode to cathode ratio, cur-  
rent density, etc., to each other. It is noted  
in this connection that we do not claim to  
be the first to propose the electroplating of  
cadmium from cyanide solutions, or the use  
20 of wholly active or wholly inactive or com-  
bined active and inactive anodes or the use  
of brightening agents in general or the par-  
ticular brightening agents referred to in the  
electroplating of cadmium. It was, of  
25 course, also known prior to our invention to  
vary the composition of the bath, the anode  
to cathode ratio, the current density etc.  
Our invention lies in the coordination of  
30 these various factors in such a way that su-  
perior results may be reliably and continu-  
ously produced.

We claim:

1. Process of electroplating with cad-  
mium which comprises electro-depositing  
35 cadmium from a sodium cadmium cyanide  
bath containing from  $\frac{1}{4}$  to 6 ounces of cad-  
mium and from  $\frac{1}{4}$  to 10 ounces of free sodium  
cyanide per gallon of bath.
2. Process of electroplating with cadmium  
40 which comprises electro-depositing cadmium  
from a sodium cadmium cyanide bath con-  
taining from  $\frac{1}{4}$  to 6 ounces of cadmium and  
from  $2\frac{1}{2}$  to 6 ounces of free sodium cyanide  
per gallon of bath.
- 45 3. Process of electroplating with cadmium  
which comprises electro-depositing cadmium  
from a sodium cadmium cyanide bath con-  
taining about 2 ounces of cadmium and  
about 5 ounces of free sodium cyanide per  
50 gallon.
5. Process of electroplating with cadmium  
which comprises electro-depositing cadmium  
from a sodium cadmium cyanide bath con-  
taining from  $\frac{1}{4}$  to 6 ounces of cadmium and  
55 at least  $2\frac{1}{2}$  ounces of free sodium cyanide  
per gallon in the presence of an anode com-  
prising metallic cadmium.

5. Process of electroplating with cadmium  
which comprises electro-depositing cadmium  
from a sodium cadmium cyanide bath con-  
taining from  $\frac{1}{4}$  to 6 ounces of cadmium and

from  $2\frac{1}{2}$  to 6 ounces of free sodium cyanide  
per gallon of bath in the presence of an  
anode comprising active and inactive mate-  
rial, the ratio of the surfaces of which lies  
65 between the limits 1 to 3 and 3 to 1.

6. Process of electroplating with cadmium  
which comprises electro-depositing cadmium  
from a sodium cadmium cyanide bath con-  
taining about 2 ounces of cadmium and  
70 about 5 ounces of free sodium cyanide per  
gallon in the presence of an anode comprising  
active and inactive surfaces, the ratio of  
which is about 45 to 55.

7. Process of electroplating with cadmium  
which comprises electro-depositing cadmium  
from a sodium cadmium cyanide bath con-  
taining from  $\frac{1}{4}$  to 6 ounces of cadmium and  
75  $\frac{1}{4}$  to 10 ounces of free sodium cyanide per  
gallon at a current density of from 4 to  
100 amperes per square foot.

8. Process of electroplating with cadmium  
which comprises electro-depositing cadmium  
from a sodium cadmium cyanide bath at a  
current density of from 4 to 30 amperes per  
80 square foot in the presence of an addition  
agent.

9. Process of electroplating with cadmium  
which comprises electro-depositing cadmium  
from a sodium cadmium cyanide solution  
90 containing from  $\frac{1}{4}$  to 6 ounces of cadmium and  
from  $2\frac{1}{2}$  to 6 ounces of free sodium cy-  
anide per gallon in the presence of an anode  
comprising metallic cadmium and an inac-  
tive conductive material at a current density  
95 of from 4 to 100 amperes per square foot.

10. Process of electroplating with cadmium  
which comprises electro-depositing cad-  
mium from a sodium cadmium cyanide solu-  
100 tion containing from  $\frac{1}{4}$  to 6 ounces of cad-  
mium and from  $2\frac{1}{2}$  to 6 ounces of free sodium  
cyanide per gallon in the presence of an  
anode comprising metallic cadmium and an  
inactive conductive material at a current  
105 density of from 4 to 30 amperes per square  
foot in the presence of an addition agent.

11. Process of electroplating with cad-  
mium which comprises electro-depositing  
cadmium from a sodium cadmium cyanide  
bath containing about 2 ounces of cadmium  
110 and 5 ounces of free sodium cyanide, using  
a combined cadmium and steel anode, the  
ratio of cadmium to steel surface of said  
anode being about 45 to 55 and the ratio of  
cathode surface to anode surface being from  
115  $1\frac{1}{2}$  to 1 to 1-1, at a current density of from  
4 to 30 amperes per square foot in the pres-  
ence of an addition agent.

In testimony whereof, we affix our signatures.

MAURICE E. LOUTH.  
ARTHUR WHITE YOUNG.